

J Farrell

Manf Tin Lined Lead Pipe

No. 74755

Patented Feb 25 1868



Witnesses

W. D. Lewis

G. B. Cushing

Inventor

John Farrell  
by Bakewell & Christie,  
his Attorneys.



# United States Patent Office.

JOHN FARRELL, OF PITTSBURG, PENNSYLVANIA.

*Letters Patent No. 74,755, dated February 25, 1868.*

## IMPROVEMENT IN THE MANUFACTURE OF TIN-LINED LEAD PIPES.

The Schedule referred to in these Letters Patent and making part of the same.

TO ALL WHOM IT MAY CONCERN:

Be it known that I, JOHN FARRELL, of Pittsburgh, in the county of Allegheny, and State of Pennsylvania, have invented a new and useful Improvement in Manufacture of Tin-Lined Lead Pipe; and I do hereby declare the following to be a full, clear, and exact description thereof.

My invention relates to the manufacture of tin-lined lead pipe, or lead pipe lined with tin or such other metal or metallic alloy or composition as may by exudation, when subject to hydraulic or other heavy pressure in a solid state, be forced through an orifice properly shaped for making pipe.

Tin-lined lead pipe has heretofore been made either by tinning the lead pipe on its inside surface by an application of melted tin, which method is liable to numerous and obvious objections, or by placing a cone-shaped ingot of tin and an ingot of lead over a core or mandrel in a cylinder, and by a plunger or ram applied to them at one end of the cylinder, forcing them out through a die or dies at the opposite end of the cylinder. The difficulties which belong to this process are serious, and hitherto have not been entirely overcome: first, the great amount of friction caused by forcing the entire body of lead and tin, under a heavy pressure, along through the cylinder, and out through dies; second, since tin is harder than lead, the tin at first is pressed out through the dies faster than the lead, so that the pipe produced will not have a tin lining of uniform thickness, the tin at first being too thick, and, consequently, toward the last too thin; third, in order to produce a perfect union between the lead pipe and its tin lining, since the two will not in a solid state perfectly unite under pressure, it is necessary that the lead be cast around and against the outer face of the tin, either before or after they are placed over the core or mandrel, but such casting is objectionable, since, as block tin melts at a lower temperature than lead, the molten lead fuses the tin to a greater or less depth, and the two mix together; fourth, the preparation of cone-shaped ingots of tin, such as are now used in manufacturing such pipe, necessitates the construction of various sizes of ingot-moulds in which to cast ingots for different-sized pipe.

To obviate these and other minor objections is the object of my invention; and the nature of it consists, first, in the construction of improved apparatus for making tin-lined lead pipe; second, in the construction of an improved compound ingot of tin and lead; third, in making the tin part of such ingot with a flanged base; and, fourth, in protecting such tin part from the effects of the molten lead by a metallic shield or cover till the lead is partially set, and then effecting a union between them by pressure.

To enable others skilled in the art to make and use my invention, I will proceed to describe its construction and mode of operation, referring for that purpose to the drawings hereto annexed, in which—

Figure 1 is a vertical sectional view of the cylinder, with its mandrel and the plunger which I employ.

Figure 2 is a similar sectional elevation of a part of my apparatus, showing my mode of making tin pipe for lining purposes.

Figure 3 is a similar sectional view, showing the use of the shield or cover to protect the tin from the heat of the melted lead.

Figure 4 is a similar view, showing in section my mode of making the tin-lined pipe.

Figure 5 is an outside view of the shield or cover.

Figures 6 and 7 are sectional views of the dies I employ.

Like letters of reference in the different figures indicate like parts.

In the cylinder *a* is bored or cast a hollow chamber, *b*, of diameter requisite for the admission and free operation of the plunger or ram *c*. Usually I find it best to make the plunger *c* stationary, and the cylinder *a* movable, but either may be made movable at pleasure. In the axis of the chamber *b* is the core or mandrel *d*, of diameter equal to the interior diameter of the pipe to be made.

The devices named being in the position shown in fig. 1, I pour into the bottom of the chamber *b* molten tin or other desirable metal or metallic alloy for lining purposes, in such quantity as may be required to form the tin pipe required for lining purposes. At or about the time that it is passing from a liquid to a solid state, or when fully solidified, I apply the plunger *c*, fitted with a die *e* of interior diameter equal to the exterior diameter of the tin pipe to be made. Then by pressure applied to either or both, the tin is forced up through the die *e* and hollow plunger *c*, till the plunger *c* reaches or nearly reaches the bottom of the chamber *b*, or till the tin is forced up on the core or mandrel *d* to the required height, when the pressing movement is arrested,

and a pipe is formed of the shape shown at *f*, fig. 2, with a flanged base, *i*. The cylinder *a* is then returned to its original position, or the plunger *e* withdrawn, as the case may be, and the shield or cover *g* of any material fusible or combustible only at a higher heat than is usually imparted to molten lead, is placed over the tin pipe *f*, fig. 3, and the rest of the chamber *b*, or any desirable part thereof, filled with melted lead, *h*. That part of the lead which comes in contact with the cover *g* is by it soon partially set or chilled, when the cover *g* is removed, and pressure is applied by the plunger *e*, or more commonly, the plunger being stationary, by the cylinder *a* to the semi-fluid lead, to cause it to unite with the tin without fusing the latter to too great a depth. When the lead has become fully solidified, or before, if so preferred, the die *e* is removed from the plunger *c*, and another die, *e'*, substituted, the interior diameter of which is equal to the exterior diameter of the lead pipe to be manufactured. Then by hydraulic or other powerful pressure, the cylinder *a* is pressed against the plunger *c*, the lead and tin forming a tin-lined lead pipe, *o*, forced out through between the die *e'* and mandrel *d*, as in fig. 4. The lead *h* in the cylinder resting on the flange *i* effectually prevents the tin *f* from being pressed out faster than is desirable. As the cylinder *a* and tin and lead move together, and the pipe is forced out at the same end at which the ram operates, friction is reduced to a minimum.

As a modification of my mode of preparing tin pipe for lining purposes, I sometimes make in the ordinary way a length of tin pipe of the requisite diameter and thickness, and cut it up into sections of length equal or about equal to the length of the core or mandrel *d*. Such sections of pipe I place over the mandrel *d*, and either cast on to them a flange, *i*, or, if so preferred, proceed with the process as above described without such flange. I do not consider the flange indispensable, though practically I find its use of great benefit in securing a tin lining of uniform thickness. Nor do I confine my invention, when a flange is used, to the particular mode described, of making the pipe *f* by pressure, as such pipe may be cast, if so preferred. If desired, the pipe *f* may be made of other metal than tin, or of a metallic alloy, provided it be not too hard to be shaped by pressure in the manner described. The shield or cover *g* I also use not only with tin pipe such as is above described, but also with tin ingots of the ordinary construction.

I thus obviate all the objections which are encountered in the ordinary process of manufacturing, as above set forth, and secure the desired results by a method which is at once simple, easy of application, certain in its operation, and by which a pipe is produced of any desirable and of a perfectly uniform thickness of tin and lead, these metals being perfectly united together, and the pipe produced being adapted to any and all uses to which such pipe is commonly applied. The wrought or pressed-tin pipe I also find better adapted to lining purposes than the ordinary cast-tin ingot.

What I claim as my invention, and desire to secure by Letters Patent, is—

1. The die *e'* in a plunger, *c*, in combination with a cylinder *a* and mandrel *d*, in a machine for making tin-lined lead pipe, constructed and operated substantially in the manner and for the purposes hereinbefore set forth.
2. The method hereinbefore described of constructing a compound ingot of tin and lead, in the manufacture of tin-lined lead pipe.
3. The use of a flange, *i*, attached to the tin part of a compound ingot of lead and tin, for the purposes and in the manner substantially as above set forth.
4. In the production of a compound tin and lead ingot by the method hereinbefore described, I claim the use of a cover, *g*, for protecting the tin pipe or tin ingot from the heat of the molten lead, substantially as and for the purposes hereinbefore set forth.

In testimony whereof, I, the said JOHN FARRELL, have hereunto set my hand, in presence of—

JOHN FARRELL.

Witnesses:

GEO. H. CHRISTY,  
A. S. NICHOLSON.